

## UNITED STATES PATENT OFFICE

HAROLD ROBERT RAFTON, OF LAWRENCE, MASSACHUSETTS, ASSIGNOR TO RAFFOLD PROCESS CORPORATION, A CORPORATION OF MASSACHUSETTS

## METHOD OF SIZING CARBONATE FILLED PAPER

No Drawing.

Application filed September 5, 1928. Serial No. 304,176.

This invention relates to a method of sizing paper and more particularly to a method of sizing paper filled with carbonate filler.

The principal object of this invention is to provide a method of sizing paper filled with carbonate filler wherein a paraffin emulsion made with a substantially water insoluble type emulsifying agent is added to a paper mix in the beater together with a fibre associating agent, and a restoring agent is added to the resulting mix at the wet end of the paper machine.

Other objects and advantages of this invention will become apparent during the course of the following description.

My invention is directed to sized paper such as is used for printing purposes for coating raw stock, or the like. It is not directed to waterproof products such as prepared roofing or the like, nor to paraffined papers which normally have a paraffin finish, which makes them substantially waterproof and usually translucent or transparent and unsuited for the uses to which I wish to put my sized paper.

I have discovered that certain grades of paper filled with carbonate filler may be sized by adding to the paper mix in the beater a paraffin emulsion made with a substantially water insoluble type emulsifying agent and a fibre associating agent preferably comprising sodium resinate and alum, and restoring the fibre associating properties of the fibre associating agent which are deteriorated, sometimes even to the point of destruction, by the carbonate filler, by adding a suitable restoring agent such as alum to the resulting mix at the wet end of the paper machine.

In the preferred practice of my process I add to fibrous material containing a carbonate filler in a beater or the like a suitable amount of a paraffin emulsion of the above referred to character. In preparing such an emulsion I may use a substantially water insoluble type emulsifying agent such as clay or even carbonate filler itself. The method of making such emulsions is well known and this method ordinarily comprises heating paraffin above its melting point and adding

the heated paraffin with vigorous agitation to a suspension of the substantially water insoluble material in water which is preferably maintained at approximately the same temperature as that of the melted paraffin. Vigorous agitation is meanwhile carried on and is continued while the emulsion is cooling. I then add to a fibrous mix in a beater, mixer or similar device, the paraffin emulsion and a suitable fibre associating agent to associate the paraffin emulsion with the fibre, said agent comprising preferably sodium resinate and alum. Preferably after the sodium resinate and alum are thoroughly mixed with the fibre I then add carbonate filler, and/or if desired, fibrous materials coming under the definition of carbonate filler hereinafter set forth. It is possible to add all the fibrous constituents and/or the carbonate filler itself in the beater prior to the addition of the alum or the sodium resinate and alum, but my experiments have indicated that better results are obtainable when the sodium resinate and alum are added to the fibre in the absence of any carbonate filler.

Moreover in furnishing the beater, I preferably use fresh water or white water which has been clarified so that the sodium resinate alum reaction may completely take place before the addition of carbonate filler in any form to the mix.

The amount of sodium resinate I may use is that amount which by itself when precipitated with alum, and restored with a subsequent quantity of alum, in accordance with my copending application Serial No. 304,168 filed Sept. 5, 1928, would not be sufficient to size the paper, but would produce a substantially unsized paper. Thus the reaction product produced by sodium resinate and alum and then subsequently restored does not in this case act as a sizing agent but as a fibre associating agent. Of course, I may, if I desire, use a greater quantity of sodium resinate, but it is to be pointed out that it is possible to secure sizing by my process where there is not enough sodium resinate used to impart sizing of itself.

I have found that the fibre associating properties of the sodium resinate and alum

re somewhat deteriorated, sometimes even to the point of destruction, by the presence of the carbonate filler before the mix is passed to the web-forming device of a paper machine. However I have discovered that the fibre associating properties of these materials may be restored by adding a suitable restoring agent such as alum preferably in solution, preferably continuously, to the mix at the wet end of the paper machine. This results in restoring the desired properties of the fibre associating agent and reassociates the emulsion with the fibre with the result that the finished paper produced from such a mix is suitably sized. If the sizing restoring agent were not employed only such parts of the paraffin emulsion as would be mechanically filtered out by the fibre would be retained thereon and the paper produced would not be satisfactorily sized, except possibly at the expense of a greatly increased quantity of paraffin, which would be undesirable because of certain mechanical instability as indicated below, as well as because of prohibitive cost.

It is necessary as indicated to add the restoring agent at or subsequent to the point of dilution of the mix, as I have found that if it is added when the mix is in relatively concentrated condition, and particularly when the relatively concentrated mix is subjected to agitation as is normal in stock chests, the restoring effect is very quickly deteriorated even to the point of complete destruction. The restoring effect even when the mix is in the diluted condition is gradually deteriorated, but is substantially unaffected within the time limits that the mix is maintained in the dilute state in the usual paper-making procedure. Moreover, although agitation in the dilute state hastens to a certain extent the deterioration of the restoring effect, the speed of deterioration is not nearly so pronounced as in the concentrated condition, and from a practical standpoint I have found that the agitation to which the diluted mix is subjected prior to delivery onto the web-forming device does not deteriorate the restoring effect to a substantial degree. In other words, the restoring agent is added at a point in the process where there is a minimum of time and intimacy of contact of the constituents of the mix.

Although clay is my preferred substantial water insoluble emulsifying agent I may use also other substantially water insoluble emulsifying agents which do not exist as such originally, such for example as any agent formed from two mutually precipitating materials which is adapted to yield a substantially water insoluble coating around the individual articles of paraffin. The method of making such emulsions is well known. Such an emulsion may be completely made prior to addition to the fibrous pulp, or it may be formed in the pulp by dispersing the paraffin origi-

nally in a soluble material which will prevent its agglomeration in the pulp mass, and then subsequently forming a substantially water insoluble coating on the dispersed paraffin particles by adding to the pulp mass and dispersed paraffin a material which will mutually precipitate the original dispersing material into a substantially water insoluble layer or film around the dispersed paraffin particles.

Papers made in accordance with my invention are sized but because of the relatively large size of the particles in comparison with the nonbreakable paraffin emulsion described in my copending applications Serial No. 304,170 filed Sept. 5, 1928, and Serial No. 304,173 filed Sept. 5, 1928, the sizing is not quite so well distributed throughout the paper. Thus it is usually desirable to use somewhat more paraffin than in the above referred to copending applications. Moreover in order to secure uniform distribution of sizing this invention may advantageously be employed in connection with the process outlined in my copending application Serial No. 304,168 of Sept. 5, 1928. However in view of the fact that the emulsifying agent employed in the practice of this invention is relatively inexpensive, an appreciable net economy results from this process. Moreover, this invention is of great advantage for preparing certain grades of paper where the requirements are not so exacting.

The emulsion herein employed, although reasonably resistant to chemical agencies, especially if the substantially water insoluble emulsifying agent employed be also substantially acid insoluble, has certain defects from a mechanical standpoint which should be taken into account in its use. The chief difficulty is that this emulsion has a tendency to be mechanically unstable, and when subjected to pressure as by the action of the beater, some of the particles may have their protective coating of clay removed, and thus be released from emulsified condition with consequent release of particles of free paraffin in the stock, which have a tendency to agglomerate and cause trouble in the paper making process. For this reason it is desirable to beat the fibre prior to the addition of the emulsion and then raise the beater roll just prior to adding the emulsion, using the roll merely for mixing rather than for beating purposes thereafter in order to prevent the breakdown of the emulsion by the beater.

The action of the fibre associating agent does not seem to have a noticeable breaking effect on the emulsion itself, and thus the paraffin is not thereby directly released from emulsion, but the same defect regarding the action of mechanical agencies on the emulsion as set forth above seems to be inherent in the emulsion whether alone, or when associated with the fibre associating agent.

An illustrative furnish which may advantageously be used in practicing my invention is as follows:

*Materials added in the beater*

|                                                                                             | Pounds |
|---------------------------------------------------------------------------------------------|--------|
| 5 Fibrous furnish (e. g. sulphite and soda pulps)                                           | 1700   |
| Rosin (added in the form of sodium resinate)                                                | 10     |
| Paraffin (added in the form of a substantially water insoluble emulsifier type of emulsion) | 40     |
| Alum (ordinary $Al_2(SO_4)_3 \cdot 18H_2O$ )                                                | 30     |
| 10 Calcium carbonate magnesium hydroxide (carbonate filler)                                 | 300    |

*Material added proportionately and continuously on dilution*

|                                                                     | Pounds |
|---------------------------------------------------------------------|--------|
| Restoring agent, e. g. alum (ordinary $Al_2(SO_4)_3 \cdot 18H_2O$ ) | 50     |

15 Another illustrative furnish is as follows:

*Materials added in the beater*

|                                                                                             | Pounds |
|---------------------------------------------------------------------------------------------|--------|
| 20 Fibrous furnish (e. g. approximately equal parts of sulphite, soda and old paper stocks) | 1800   |
| Rosin (added in the form of sodium resinate)                                                | 10     |
| Paraffin (added in the form of a substantially water insoluble emulsifier type of emulsion) | 35     |
| Alum (ordinary $Al_2(SO_4)_3 \cdot 18H_2O$ )                                                | 30     |
| Calcium carbonate magnesium hydroxide (carbonate filler)                                    | 200    |

*Material added proportionately and continuously on dilution*

|                                                                        | Pounds |
|------------------------------------------------------------------------|--------|
| 25 Restoring agent, e. g. alum (ordinary $Al_2(SO_4)_3 \cdot 18H_2O$ ) | 50     |

In the above formula, the weights of carbonate filler refer to bone dry basis, the weights of all other ingredients being given on the air dry basis.

In regard to the paraffin used, it is to be understood that either low or high melting point material can be employed. The so-called fully refined paraffin is entirely satisfactory since it does not impart objectionable color to white sheets. However, for purposes of economy, it is often desirable to use a less pure material such for example as the material which is commonly known to the trade as semi-refined paraffin scale, containing approximately 1-2 per cent. of oil and water as impurities, which material gives satisfactory results. Such material will perhaps in certain cases have varying melting points but one particular sample used, for example, had a melting point of approximately 115° F. (46° C.). Other even more impure paraffins may be used, especially if the color (whiteness) requirements of the finished paper are not too exacting, or if papers, other than white, are to be made.

In place of alum in the practice of my process, both as originally added in the beater and as a restoring agent, I may employ with a measure of success an acid such as sulfuric acid ( $H_2SO_4$ ), an acid salt such as sodium bisulfate ( $NaHSO_4$ ), or a salt of a trivalent metal, such as ferric iron or the other salts of aluminum. Of the aluminum salts available I may use the chloride or the like, but I prefer to use ordinary "alum".

In place of sodium resinate I may use satisfactorily in the practice of my process other soaps, such as the oleates, or any partially or

completely saponified material, such as saponified beeswax.

By the term "carbonate filler" as employed herein, is intended to be included calcium carbonate, of which lime mud from the causticizing process is one form; calcium carbonate magnesium basic carbonate employed in the paper disclosed in my U. S. Patent No. 1,595,416; calcium carbonate magnesium hydroxide disclosed in my U. S. Patent No. 1,415,391; or other substantially water insoluble normal or basic carbonates of alkaline earth metals, (which expression is herein intended to include magnesium), or compounds, double salts, or physically associated mixtures of these with one or more other acid soluble materials of a substantially water insoluble nature. The term "carbonate filler" is also intended to include fibrous material and/or other material such as paper coating constituents or the like containing one or more compounds of the character referred to, such as "old papers" or similar papers, "broke", or the like.

By the term "wet end of the paper machine" is intended to be included those instrumentalities employed in paper manufacture by which and/or in which a relatively concentrated paper mix is diluted, and treated, conveyed or fed up to the point of web-formation, such as the mixing box, regulating and proportioning devices, riffles, troughs, screens, head boxes, inlets, and the like, including also instrumentalities used in the white water cycle.

When I employ the term "paraffin" herein, I mean paraffin wax, which is solid at ordinary or room temperature. I do not mean to restrict myself only to the paraffin hydrocarbons, but mean to include in this term all the hydrocarbons of a waxy nature substantially unsaponifiable and inert to acidic and alkaline materials under ordinary conditions of temperature and pressure, whether derived from petroleum, shale, lignite, earth wax, or other natural or artificial sources. I do not, however, mean to include in this term material of a pitchy nature, such as bitumen or asphalt.

Where I use the term "sodium resinate" it is to be understood that I mean it to include any material produced by the action of alkali, generally in aqueous solution, on rosin, or on natural or synthetic resin acid or acids, regardless of the exact composition of the product, or the varying composition which different samples may possess.

When I use the word "paper" herein, I use it in the broad sense to include products of manufacture of all types and of all weights and thicknesses, which contain as an essential constituent a considerable amount of prepared fibre and which are capable of being produced on a Fourdrinier, cylinder, or other

forming, felting, shaping or molding machine.

While I have described in detail the preferred embodiment of my invention, it is to be understood that the details of procedure, the proportions of ingredients, and the arrangement of steps may be widely varied without departing from the spirit of the invention or the scope of the subjoined claims.

I claim:

1. The method of sizing paper filled with carbonate filler comprising mixing with fibrous material a paraffin emulsion made with substantially water soluble type emulsifying agent, fibre associating agent, and carbonate filler, and thereafter adding a restoring agent under conditions favoring the minimizing of the time of contact of the constituents of the mix, and thereafter making paper therefrom.

2. The method of sizing paper filled with carbonate filler comprising mixing with fibrous material a paraffin emulsion made with substantially water insoluble type emulsifying agent, fibre associating agent, and carbonate filler, and thereafter adding a restoring agent under conditions favoring the minimizing of the intimacy and time of contact of the constituents of the mix, and thereafter making paper therefrom.

3. The method of sizing paper filled with carbonate filler comprising mixing with fibrous material a paraffin emulsion made with substantially water insoluble type emulsifying agent, fibre associating agent, and carbonate filler, and thereafter adding a fibre associating restoring agent under conditions favoring the minimizing of the intimacy and time of contact of the constituents of the mix, and thereafter making paper therefrom.

4. The method of sizing paper filled with carbonate filler comprising mixing with fibrous material a paraffin emulsion made with substantially water insoluble type emulsifying agent, fibre associating agent, and carbonate filler, and thereafter adding a sizing restoring agent under conditions favoring the minimizing of the intimacy and time of contact of the constituents of the mix, and thereafter making paper therefrom.

5. The method of sizing paper filled with carbonate filler comprising mixing with fibrous material a paraffin emulsion made with substantially water insoluble type emulsifying agent, fibre associating agent, and carbonate filler, and thereafter adding a restoring agent at the wet end of the paper machine.

6. The method of sizing paper filled with carbonate filler comprising mixing with fibrous material a paraffin emulsion made with substantially water insoluble type emulsifying agent, carbonate filler, and fibre associating agent comprising saponified material and precipitant therefor, and thereafter adding to the resulting mix a salt of a trivalent metal at the wet end of the paper machine.

7. The method of sizing paper filled with carbonate filler comprising mixing with fibrous material a paraffin emulsion made with a substantially water insoluble type emulsifying agent, carbonate filler, and fibre associating agent comprising saponified material and a salt of a trivalent metal, and thereafter adding to the resulting mix a restoring agent for said fibre associating agent at the wet end of the paper machine.

70 7. The method of sizing paper filled with carbonate filler comprising mixing with fibrous material a paraffin emulsion made with a substantially water insoluble type emulsifying agent, carbonate filler, and fibre associating agent comprising saponified material and a salt of a trivalent metal, and thereafter adding to the resulting mix a restoring agent for said fibre associating agent at the wet end of the paper machine.

8. The method of sizing paper filled with carbonate filler comprising mixing with fibrous material a paraffin emulsion made with a substantially water insoluble type emulsifying agent, carbonate filler, and fibre associating agent comprising saponified material and a salt of aluminum, and thereafter adding to the resulting mix a restoring agent for said fibre associating agent at the wet end of the paper machine.

85 9. The method of sizing paper filled with carbonate filler comprising mixing with fibrous material a paraffin emulsion made with a substantially water insoluble type emulsifying agent, carbonate filler, and fibre associating agent comprising saponified material and alum, and thereafter adding to the resulting mix a restoring agent for said fibre associating agent at the wet end of the paper machine.

90 10. The method of sizing paper filled with carbonate filler comprising mixing with fibrous material a paraffin emulsion made with a substantially water insoluble type emulsifying agent, carbonate filler, and fibre associating agent comprising sodium resinate and alum, and thereafter adding to the resulting mix a restoring agent for said fibre associating agent at the wet end of the paper machine.

100 11. The method of sizing paper filled with carbonate filler comprising mixing with fibrous material a paraffin emulsion made with a substantially water insoluble type emulsifying agent, carbonate filler, and fibre associating agent comprising a saponified material and precipitant therefor, and thereafter adding to the resulting mix a salt of a trivalent metal at the wet end of the paper machine.

110 12. The method of sizing paper filled with carbonate filler comprising mixing with fibrous material a paraffin emulsion made with a substantially water insoluble type emulsifying agent, carbonate filler, and fibre associating agent comprising saponified material and precipitant therefor, and thereafter adding to the resulting mix a salt of aluminum at the wet end of the paper machine.

120 13. The method of sizing paper filled with carbonate filler comprising mixing with

75

80

85

90

95

100

105

110

115

120

125

130

fibrous material a paraffin emulsion made with a substantially water insoluble type emulsifying agent, carbonate filler, and fibre associating agent comprising saponified material and precipitant therefor, and thereafter adding to the resulting mix alum at the wet end of the paper machine.

14. The method of sizing paper filled with carbonate filler comprising mixing with fibrous material a paraffin emulsion made with a substantially water insoluble type emulsifying agent, carbonate filler, sodium resinate, and alum, and thereafter adding to the resulting mix alum at the wet end of the paper machine.

15. The method of sizing paper filled with carbonate filler comprising mixing with fibrous material a paraffin emulsion made with a substantially water insoluble type emulsifying agent, carbonate filler, and fibre associating agent comprising saponified material and precipitant therefor in an amount insufficient of itself to impart substantial sizing to the paper, and thereafter adding to the resulting mix a restoring agent for said fibre associating agent at the wet end of the paper machine.

16. The method of sizing paper filled with carbonate filler comprising mixing with fibrous material a paraffin emulsion made with a substantially water insoluble type emulsifying agent, carbonate filler, sodium resinate in an amount insufficient of itself to impart substantial sizing to the paper, and alum, and thereafter adding to the resulting mix alum at the wet end of the paper machine.

17. In a method of the character described, the step of adding a restoring agent at the wet end of the paper machine.

18. In a method of the character described, the step of adding a salt of a trivalent metal at the wet end of the paper machine.

19. In a method of the character described, the step of adding alum at the wet end of the paper machine.

In testimony whereof I affix my signature.  
HAROLD ROBERT RAFTON.

**CERTIFICATE OF CORRECTION.**

Patent No. 1,803,651.

Granted May 5, 1931, to

**HAROLD ROBERT RAFTON.**

It is hereby certified that error appears in the printed specification of the above numbered patent requiring correction as follows: Page 4, line 14, claim 1, for the word "soluble" read insoluble; and that the said Letters Patent should be read with this correction therein that the same may conform to the record of the case in the Patent Office.

Signed and sealed this 4th day of August, A. D. 1931.

Wm. A. Kinnan,  
Seal) Acting Commissioner of Patents.